

Jan. 1, 1924

1,479,044

L. KIRSCHBRAUN

COMPOSITE BOARD AND PROCESS OF MAKING SAME

Filed Aug. 16. 1922



witness:

Stephen A. Pebara

Inventor:  
Lester Kirschbraun

by Frank L. Belknap. Aug.

## UNITED STATES PATENT OFFICE.

LESTER KIRSCHBRAUN, OF CHICAGO, ILLINOIS.

## COMPOSITE BOARD AND PROCESS OF MAKING SAME.

Application filed August 16, 1922. Serial No. 582,310.

*To all whom it may concern:*

Be it known that I, LESTER KIRSCHBRAUN, a citizen of the United States, residing in the city of Chicago, county of Cook, State of Illinois, have invented certain new and useful Improvements in Composite Board and Processes of Making Same, of which the following is a specification.

This invention relates to improvements in boards and is particularly advantageous in the manufacture of wall-boards. One of the objects of the invention is to produce a structure which is very strong and stiff and will not take up moisture and be subject to expansion, contraction or abutment.

The invention may be carried out as follows:

An emulsion of asphalt, colloidal clay and water may first be formed in the manner described in my prior Patent No. 1,417,835. This emulsion may then be mixed with fibre. To this mixture may then be added infusorial or diatomaceous earth. The emulsion is preferably relatively thick and pasty, of a character such as comes from the emulsifier and prior to any dilution by water. To this emulsion of asphalt clay and water may be added dry fibre. This dry fibre is thoroughly macerated in the emulsion and the dry fibre takes up or soaks up water from the emulsion. This of course makes a thicker mixture than the emulsion alone. To this mixture or simultaneous with the addition of the fibre is added dry infusorial earth in more or less powdered form. This dry earth is thoroughly mixed with the other ingredients and it will take up still more water and still further thicken the mass. The result is to produce a more or less pulverulent granular composition without much cohesion and of such a consistency that it can be loosely and readily spread in a sheet or other form.

The percentages of the various ingredients may for example be as follows:

The final composition may have about three to five parts of fibre, forty-five parts of infusorial earth, ten parts of clay and forty parts of asphalt, all by weight. It is understood, however, that these percentages may be varied widely.

The composition thus formed may then be spread over a sheet of paper mounted on a table or other movable support and a second layer of paper placed on the top of the sheet

thus formed, and the three layers, i. e., the two layers of paper and the layer of the composition above described pressed together to form a unitary structure, it being understood that the outer layers of paper will firmly adhere to the inner composition layer.

During the pressing operation it may be desirable to more effectively remove water. The outer layers of paper may be 15 to 30 points caliper and the inner-midst composition layer may be seventy-five to one hundred and twenty-five points caliper.

An invention may be carried out in which the fibre may be materially reduced or entirely dispensed with.

An invention may be carried out in the manner first described in which, instead of using infusorial earth, ground cork, sawdust, or a mixture of both and with or without infusorial earth may be used. It may be here stated that it is desirable to produce a board that is not merely strong and weather resisting as above referred to, but is also light in weight.

In carrying out the invention or inventions in any of the manners above described, it is desirable that the composition when sheeted, be subjected to high pressure in order to consolidate it and make as dense a product as possible. Also, it may be desirable to run the formed sheet through steam-heated rollers to effectively remove all moisture, but it may be noted that the percentage of water in the final composition is, relative to the other constituents, relatively small. In fact the mixture might be air-dried before it is sheeted so as to reduce the water content to a minimum.

It is to be noted that it is desirable to use a pitch of sufficiently hard character, as for example, asphalt to from 160° Fahrenheit to 175° Fahrenheit and such a percentage of colloidal clay so as to produce a sufficiently fine dispersion to the asphalt as to permit a relatively large percentage of the water being transferred to the fibre and infusorial earth without breaking down the emulsion and making an undesirable gummy mass.

Instead of making wallboard in the manner above described, a linoleum-like product may be formed in which the composition referred to is spread over burlap and pressed thereto and then dried as heretofore described. This results in making an imper-

meable wear-resisting surface, capable of being painted or otherwise colored, but in such case it may be desirable to use for example, linseed or other oxidizable oil bases instead of asphalt.

I claim as my invention:

1. A waterproof board consisting of a plurality of plies, one of said plies consisting essentially of bitumen or pitch, infusing .0 rial earth and fibre.
2. A waterproof board consisting of a plurality of plies, one of said plies consisting essentially of bitumen or pitch, and in- fusorial earth.
3. A board consisting of outer plies and an inner core, said inner core containing bitu-

men, fibre and a light-weight porous material.

4. A process of making a board consisting in forming an emulsion of pitch, clay and water, macerating in said emulsion relatively dry fibre and dry porous material, and forming this composition into a sheet between two outer covering plies.

5. A process of making a board consisting in making an emulsion of bitumen or pitch, water and an emulsifying agent adding thereto relatively dry fibre and infusorial earth and forming this composition into a sheet between two outer covering plies.

LESTER KIRSCHBRAUN.